

March 12, 1940.

G. CHARLTON

2,193,088

POPPET VALVE BLANK AND METHOD OF MAKING SAME

Original Filed June 28, 1937



INVENTOR  
George Charlton.  
BY  
Harness, Dickey & Pierce.  
ATTORNEYS.

## UNITED STATES PATENT OFFICE

2,193,088

POPPET VALVE BLANK AND METHOD OF  
MAKING SAME

George Charlton, Battle Creek, Mich., assignor to  
Eaton Manufacturing Company, Cleveland,  
Ohio, a corporation of Ohio

Original application June 28, 1937, Serial No.  
150,771. Divided and this application Febru-  
ary 12, 1938, Serial No. 190,220

## 6 Claims. (Cl. 29—156.7)

This invention relates to poppet valves and to a method of making the same and is particularly adaptable for use in connection with poppet valves of the type employed in internal combustion engines and to those types thereof which are hollow and contain sealed therein a mass of coolant material. This application is a division of my application for Letters Patent of the United States filed the 28th day of June, 1937 for improvements in Valve structure and method of forming, Serial No. 150,771.

Objects of the invention include the provision of a new and novel method of forming a hollow poppet valve; the provision of a novel method of making a hollow poppet valve formed from a plurality of independently formed parts; the provision of a method of making hollow poppet valves in which the head portion and the stem portion of the valve are independently formed and are thereafter joined by internally distributing a mass of molten metal under the effects of centrifugal force over the joint between them; the provision of a method of making a hollow poppet valve in which the head portion of the valve is independently formed from the stem portion thereof and both portions thereof are hollow, so forming the stem portion as to predetermine its position with respect to the head portion when initially assembled thereto, temporarily securing the two portions together in sealed relationship, and then distributing a mass of molten metal to the joint between the parts under the effects of centrifugal force, and thereafter machining the structure to bring it to its completed size, shape and contour; and the method of making a hollow poppet valve as above described in which the molten metal employed for bonding the two parts together is initially introduced into one of the parts in solid state and both parts are thereafter heated to a sufficient temperature to effect a melting of the bonding material without effecting a melting of the parts.

Further objects include the provision of a novel form of poppet valve blank; and the provision of a poppet valve blank constructed of a plurality of separately formed parts so initially formed as to predetermine their assembled relationship when assembled together.

The above being among the objects of the present invention the same consists in certain novel features of construction, combination of parts, and step or steps of operation to be herein-after described with reference to the accompanying drawing, and then claimed, having the above and other objects in view.

In the accompanying drawing which illustrates suitable embodiments of the present invention, and in which like numerals refer to like parts throughout the several different views,

Fig. 1 is a vertical sectional broken view taken axially through the stem portion of a valve constructed in accordance with the present invention as initially formed independently of the head portion and before its assembly to the head portion;

Fig. 2 is an axial view of the valve stem shown in Fig. 1 taken as on the line 2—2 of Fig. 1;

Fig. 3 is a vertical sectional view taken axially through an independently formed head portion of a valve to be constructed in accordance with the present invention prior to the assembly of the stem portion thereto;

Fig. 4 is a fragmentary sectional view taken axially through the parts and illustrates the stem portion shown in Fig. 1 assembled to the head portion shown in Fig. 3 and welded thereto to temporarily seal the joint between them and maintain them in a predetermined position, a mass of the material which is to be employed to bond the two parts together being shown as contained within the bottom of the hollow interior of the stem portion;

Fig. 5 is a view similar to Fig. 4 after the bonding operation has been completed;

Fig. 6 is a partially broken vertical sectional view taken axially through a completed valve formed in accordance with the disclosure in the preceding figures;

Fig. 7 is a fragmentary vertical sectional view taken centrally through the head portion of a valve similar to that shown in Fig. 6 but including certain additional features;

Fig. 8 is a view similar to Fig. 4 but illustrating a modified form of construction; and,

Fig. 9 is a fragmentary vertical sectional view taken axially through a completed valve formed in accordance with the disclosure in Fig. 8.

The invention may be employed for integrally uniting a plurality of parts to form an integral valve structure. In such case the plurality of parts are so constructed and arranged as to provide a reservoir for a granular alloy material and the parts are so constructed and arranged that upon melting of the material and spinning of the assembly the alloying material will become distributed in the joint between the parts and after solidifying will form all of the parts into a unitary valve structure. Accordingly, the invention is particularly valuable in connection with the forming of hollow valves and particularly hollow

valves of the type adapted to enclose a suitable amount of metallic sodium or other suitable material which will melt or will remain fluid when the valve is operating at elevated temperatures 5 and will serve to carry the heat away from the head portion thereof to the stem portion and dissipate it through parts in contact with the stem portion in accordance with known practices.

In such case the valve is made up initially of 10 a hollow head portion and an independently formed hollow stem portion the character of both of which is such as to permit them to be easily and quickly machined. The stem portion in such case is initially formed in such a manner as to provide a space adjacent the joint between the parts when assembled together for receiving the alloying or other material which is to form a bond between the parts. The stem portion and the head portion are then assembled together, 15 temporarily secured together in assembled relationship and the joint between them temporarily sealed, the bonding material is introduced into the stem portion and then both portions are heated to a temperature sufficient to melt the bonding material without causing a melting of the head portion and the stem portion and while the bonding material is in molten condition the assembly is subjected to a spinning operation whereby the molten material under centrifugal 20 force is distributed to the joint between the parts where it bonds itself to both parts, seals the joints between the parts and permanently secures the parts together in such a manner as to effectively prevent leakage or escape of a contained cooling 25 medium when employed from the interior of the valve during operation of the valve under high 30 temperatures.

It has heretofore been suggested that hollow 35 valves intended to contain sodium or other cooling agent be formed by constructing the valve in two or more pieces each of which may be relatively easily machined, and thereafter welding them together by known methods as, for instance, electric or gas welding, but this practice has 40 never become commercially practicable for the reason that it is commercially impracticable in production to produce valves in this manner without an unduly large percentage of scrap, and the final product, even where the weld appears perfect, too frequently develops cracks in the welded 45 zone which permits escape of the contained cooling medium. Because of these reasons such types of valves as have heretofore been successfully used commercially and produced in commercial 50 quantities have each been produced from a single piece of steel by boring it out of a solid bar and swaging down the portion desired for the stem to suitable dimensions, which obviously requires 55 an unusually large amount of extremely careful and expensive work in its production. By the 60 employment of the present invention the most difficult parts of the valve structure may be easily, quickly and economically produced on screw machines and the bond produced between the various independently formed parts is of such a character as to definitely eliminate the production 65 of any valves of this type which require scrapping because of the defects in the weld or bond, or weakness in the bonded zone.

70 Referring now to the drawing which shows preferred methods of manufacturing a valve in accordance with the present invention and valves constructed in accordance therewith, and referring first to the construction illustrated in Figs. 1 to 6, inclusive, the independently formed

stem portion of the valve is illustrated in Figs. 1 and 2. In these figures the stem portion is indicated generally at 10 as comprising a hollow cylindrical body having a bore 11, a closed end 12 and an open end 14. The diameter of the body 10 over the greater portion of its length is slightly greater than the outside diameter desired in the finished valve stem. The end 14 is initially made of a materially greater diameter as illustrated so that during the final steps of operation 10 this end may be swaged down to bring the outer diameter commensurate with the diameter of the main body portion of the stem and thereby constrict the bore of the stem in the manner illustrated at 16 for reasons which will hereinafter be 15 more apparent. On its outer face the closed end 12 is provided with an axial projection 17 the purpose of which will hereinafter be apparent and the side walls of the main body portion 10 of the stem immediately above the end wall 12 are provided with one or more radial apertures 18 there-through.

The head portion 20 of the valve which is shown in Fig. 3 is initially formed as a short cylindrical block of slightly greater diameter than 25 that desired for the finished head and is provided with an axial bore 22 extending thereinto from one end of a diameter slightly larger than the diameter of the main body portion of the stem 10 so as to enable the same to be received therein, 30 and an enlarged bore or pocket portion 24 positioned concentrically with respect to the axis of the head 20 and in open communication with the bore 22. It may be desirable in some cases to provide an annular groove such as 26 centrally 35 of the length of the bore 22 as shown.

The above portions of the valve and particularly the head portion 20 may be made from any suitable steel or steel alloy such as is commonly used for the valves of internal combustion 40 engines. Where the valve is to be used as an exhaust valve these portions of the valve are preferably of a type of steel that will stand the high temperatures and corrosive action of the 45 exhaust gases and in such case it may be desirable to employ an alloy generally known to the trade as silichrome X-142 having approximately the following analysis. This alloy has a melting point of approximately 2650° F.

|            |                  |    |
|------------|------------------|----|
| Carbon     | 40% to .50%      | 50 |
| Manganese  | .70% maximum     |    |
| Chromium   | 13.00% to 15.00% |    |
| Nickel     | 13.00% to 15.00% |    |
| Silicon    | .30% to .30%     |    |
| Tungsten   | 1.75% to 3.00%   | 55 |
| Phosphorus | .03% maximum     |    |
| Sulphur    | .03%             |    |
| Iron       | Remainder        |    |

Another suitable alloy for use in the head 20 and stem 10 is as follows, the percentages given being approximate.

|           | Per cent         |    |
|-----------|------------------|----|
| Carbon    | .75              | 65 |
| Manganese | .50              |    |
| Chromium  | 19.00            |    |
| Nickel    | 1.75             |    |
| Silicon   | 2.25             |    |
| Balance   | Principally iron | 70 |

This alloy has a melting point of approximately 2600° F. The first of these alloys is known as an austenitic type of alloy, and does not become hard upon heating and quenching. The last described alloy is known as a hardening type of 75

alloy; that is, it becomes hard upon heating and quenching. These two alloys are set out merely as illustrative of the various types of material that may be satisfactorily employed for the head 5 and stem 10.

As will be apparent to those skilled in the art the stem 10 and head 20 are of such character that they may be readily formed from bar stock on screw machines or the like in a quick, easy 10 and economical manner. On the other hand they may be formed in any suitable or desirable manner and the head in particular formed by suitable initial forging or other operations. In any case the hollow interiors of both the head and 15 the stem portions will be readily available to easy machining operation so as to bring their internal dimensions to accurate conformance with a predetermined standard of size, shape and contour.

After the stem 10 and head 20 have been initially and independently formed to the condition illustrated in Figs. 1 and 3 the same are then assembled to one another in the manner illustrated in Fig. 4. In other words that end of the stem 10 including the end wall 12 is inserted into 25 the bore 22 of the head 20 until the projection 17 bottoms against the end wall of the pocket 24 in the manner illustrated in Fig. 4. It will thus be apparent that the projection 17 serves as a means for locating the stem 10 in axially desired relation 30 with respect to the head 20. Accordingly, the length of the projection 17 may be so governed as to obtain any desired relationship between the head and the stem but in the particular instance shown this is such as to bring the radial openings 35 18 in the stem 10 to radial alignment with the annular groove 26 in the head 20. In the figures the amount of clearance between the outer surface of the stem 10 and the bore 22 of the head 20 is exaggerated in order to better illustrate the 40 construction, it being understood that in actual practice the fit between these parts will be sufficiently close that while it permits a complete distribution of the bonding material over the entire joint between the parts this bonding layer 45 will not be of excessive thickness. In some cases at least it may be found satisfactory to so control the clearance between these parts that it will effect a capillary action on the bonding material tending to draw the bonding material throughout 50 the entire area of the joint between the parts. However, due to the spinning operation herein-after described it will be understood that such capillary attraction of the bonding material is not entirely relied upon to obtain the proper distribution of the bonding material throughout the 55 area of the joint.

The parts being assembled as illustrated in Fig. 4 they are then welded together as at 28, preferably by gas or electric welding, not only to temporarily secure these parts together in assembled relationship but also to seal this end of the joint between the parts against the escape of the bonding material during the step of distributing this material between the parts.

When the parts have reached the stage of assembly illustrated in Fig. 4 a mass of material 30 which it is desired to employ as the agent for bonding the two parts together is then deposited in the bottom of the stem portion 10 as illustrated in Fig. 4. The material 30 will usually be of a composition which will be determined to a great extent by the use to which the valve is to be put. Where the valve is not to be employed in internal combustion engines and is 70 not to be employed for any use which will re-

quire it to withstand anything above normal room temperatures, or relatively low temperatures, it may be hard solder, spelter or the like. Where higher temperatures are to be encountered by the valve any suitable metal or alloy 5 capable of being bonded to the head 20 and stem 10 in molten condition and of such a character as to stand the temperatures to be encountered without melting or materially weakening its structure may be employed. Aluminum bronze is 10 an example of a material that may be employed under such conditions. Where the valve is for an internal combustion engine and particularly where it is of the sodium or other internally cooled type requiring it to withstand relatively 15 high temperatures, and the stem and head of the valve are formed from a suitable steel or steel alloy such as those heretofore specifically set out, a suitable alloy having a melting point lower than that of the head and stem of the valve 20 but nevertheless approaching the melting point of these parts will usually be found preferable. An alloy of the following composition has been found suitable for use in such case.

|           | Per cent         |
|-----------|------------------|
| Carbon    | 0.76             |
| Manganese | 0.14             |
| Chromium  | 9.04             |
| Silicon   | 0.63             |
| Nickel    | 33.17            |
| Boron     | 1.87             |
| Balance   | Principally iron |

The melting point of this alloy is approximately 2075° F. With this alloy spinning can readily be 35 done between 2150° F. and 2200° F. and it may be employed where the head and stem portions of the valve are made of any suitable type of steel having an ordinary melting point.

Another alloy suitable for use as the material 30 where the head and stem portion of the valve 40 are formed from either ordinary steel or of a steel alloy such as either of the first two analyses given as is follows:

|          | Per cent         |
|----------|------------------|
| Carbon   | 0.38             |
| Silicon  | 0.23             |
| Chromium | 14.53            |
| Tungsten | 18.08            |
| Boron    | 3.5              |
| Balance  | Principally iron |

The melting point of this alloy is approximately 2130° F. and successful spinning has been done with it at 2250° F.

One type of alloy which is marketed under a well known trade-name is also adaptable for use as the material 30. Such material is manufactured in different grades any one of which may be found suitable for use as the material 30 and as indicative of the various grades of such material the approximate analysis of one grade is here 55 set out.

|          | Per cent |
|----------|----------|
| Carbon   | 2.13     |
| Chromium | 27.36    |
| Silicon  | 1.09     |
| Tungsten | 15.33    |
| Cobalt   | 50.00    |

The melting point of this particular alloy is approximately 2350° F. Other grades of the 70 same type of alloy contain the same elements but in different proportions than those stated, the characteristics of the final product being somewhat varied thereby.

The amount of material 30 that is placed with- 75

in the stem 10 of the parts as brought to the assembled condition illustrated in Fig. 4 is preferably only slightly in excess of that required to effect the desired bond between the parts, a slight excess being provided to insure the completeness of this bond and the bulk of the excess which escapes into the pocket 24 is evenly distributed around the periphery thereof in the final product and offers no particular problem, nor is its presence particularly undesirable.

While in the broader aspects of the present invention the stem 10 and head 20 after being welded together as at 28 in Fig. 4 may be brought up to a temperature approaching or in excess of the melting point of the material 30 before the material 30 is added and in such conditions the material 30 may be added in molten condition, it is preferable to add the material 30 in granular or other suitable form as a solid material and while the assembly is at ordinary room temperature. The whole assembly including the material 30 is then placed within a suitable oven, furnace or other heating device, with the head down and the stem pointed upwardly, with the addition of a suitable flux if thought necessary, or in a neutral or non-oxidizing atmosphere, and the entire assembly is then heated to such a temperature as to effect a melting of the material 30 but not sufficiently high to effect a melting of the material from which the stem 10 and head 20 are formed. Preferably the temperature will be approximately 100 degrees in excess of the melting point of the material 30. In the absence of a furnace or other heating device not capable of heating the assembly up in a neutral or non-oxidizing atmosphere, a suitable material may be introduced into the interior of the hollow stem prior to the heating operation to prevent oxidization of the interior surfaces thereof during such operation. Alcohol is an example of such material and in such case it will be preferable to temporarily substantially close the open end of the stem during the heating operation so as to insure the maintenance of the non-oxidizing atmosphere within the hollow interior of the parts.

As soon as the parts 10 and 20 and the material 30 have been brought to a sufficient temperature to effect a melting of the material 30, the assembly is then removed from the heating device and is immediately subjected to a spinning operation about the axis of the parts. This spinning operation places the molten material 30 under a centrifugal force which drives the material 30 radially outwardly through the openings 18 and into the joint formed by the bore 22 and the opposed outer face of the stem 10, filling the groove 26 and causing this material to be intimately bonded to both the stem 10 and head 20. In some instances where the fit between the parts permits, the capillary attraction afforded by the fit as previously mentioned may aid in the distribution of the material 30 throughout the area of the joint. Also a portion of the molten material 30 will be discharged during the spinning operation into the pocket 24 where it will be distributed to the radially outer wall thereof as indicated at 32 in Fig. 5, this, of course, being unnecessary but occurring only because of the precaution taken to insure sufficient material 30 in all cases to complete the bond at the joint between the parts. Some of the material 30 will remain in the openings 18 and it will, of course, completely fill the annular groove 26 so that those portions of the material 30 remaining in the openings 18 and received in the groove 26 will serve to provide keys formed from the material

30 tending to lock the stem 10 and head 20 against axial separation by a mechanical interconnection as well as by the bond of the material 30 to these parts.

Although it will be found that a most satisfactory bond between the material 30 and the stem and head 20 will occur even though the material 30 has a melting point materially lower than the melting point of the stem 10 and the head 20, where the material 30 is formed from the higher melting point alloys, the composition of which has been specifically set out above, the temperature to which it is necessary to heat the parts to obtain the melting of the material 30 and the desired fluidity thereof for the spinning operation will often cause a sweating of the surfaces of the stem 10 and head 20 as commonly occurs preliminary to the actual melting of the material from which they are formed and where the molten material 30 is distributed to these sweating surfaces it has been found that an actual alloying of the material 30 with the material of the stem 10 and head 20 occurs so that in such case a most permanent and effective bond is established between the stem and the head which not only effectively prevents any possibility of separation of the parts in service but additionally provides a most effective seal against the escape of pressure through the joint between these parts. This feature is particularly important in connection with these valves when they are employed as internally cooled self-contained coolant types of valves subject to hard usage at elevated temperatures in internal combustion engines and particularly where they are employed as exhaust valves in the engines of airplanes, busses, trucks and the like.

The spinning operation is maintained until the material 30 has been permitted sufficient time to insure proper distribution throughout the joint between the parts and sufficient time has elapsed to permit such material 30 to solidify. Thereafter the spinning operation is terminated, the assembly is allowed to cool and is then subjected to further operations to bring it to a completed state. The first of these operations is to remove the end wall 12 and projection 17. This may be readily done by projecting a drill down the bore 11 of the stem 10 and simply drilling out the end wall 12 upon which the projection 17 may be readily discharged from the bore of the stem. This operation places the bore 11 of the stem 10 in open communication with the pocket 24 and the head 20 as illustrated in Fig. 6. The next operation may consist of swaging down the opposite end of the stem 10 as at 16 previously described to restrict its bore, as illustrated in completed form in Fig. 6, and then the exterior surfaces of the assembly thus provided may be machined to bring it to completed condition and to form a desired seating surface such as 34 on the head 20, during which operations the welded material 28 will usually be removed completely.

It may be noted that it is only when the valve is to be of the internally cooled type and in which the internal coolant is self-contained that it is necessary to constrict the bore at the upper end of the stem 10 as illustrated, but under such circumstances the restricted end of the stem 10 is then drilled and reamed out for reception of a tapered pin such as 36. Before insertion of the pin 36 the internal coolant illustrated in Fig. 6 at 38 is introduced into the hollow interior of the valve through the restricted bore in the end of the stem provided for the reception 76

of the pin 36, the pin 36 is introduced and driven firmly into place, the end of the stem 10 and pin 36 are then finished off in flush relationship, and a valve stem end portion such as 38 is then 5 welded in place on the end of the stem over the pin 36. These last precautions are taken to absolutely insure the closing of the corresponding end of the stem 10 in order to thereafter obviate any possibility of the escape of the coolant 38 10 therethrough. The finish machining operations on the valve may then be accomplished to bring the valve to its completed condition.

The material 38 which is preferably employed as the internal self-contained coolant for the 15 valve may be metallic sodium or other suitable material such, for instance, as disclosed in U. S. Patent No. 1,670,965, such material being fluid at ordinary temperatures to which such valves are subjected in normal operation of internal 20 combustion engines and which, in being continuously transferred between the stem and head portions of the valve during operation tend to carry the heat away from the head 20 to the stem 10 from which it is dissipated by contact with the 25 valve guide (not shown) or other parts in which the stem 10 is commonly in contact.

In Fig. 7 a slight modification of the above described valve is shown. In this construction, inasmuch as the modification involves only a 30 small change in the stem 10, the parts are indicated by the same numerals as employed in Figs. 1 to 6, inclusive, except such numerals bear a prime mark. The head 20' is identical to the head 20 previously described. The only difference in the stem 10' is that the exterior surface of the stem 10' in line with the radially outer ends of the openings 17' is provided with a circumferential groove 40 which lies in opposed relationship with respect to the annular groove 26'. Accordingly, in the final product the material 30' in the grooves 26' and 40 combine to form an annular ring of the material 30 between the stem 10' and the head 20' which serves to provide a more efficient mechanical interlocking between these parts. In other words this annular ring of material 30' serves as an annular key 45 between the stem 10' and head 20' mechanically interlocking these parts against axial separation.

It is not to be understood, however, that use 50 of any construction which will provide a mechanical interlocking of the two parts of the valve against axial separation is necessary in accordance with the broader aspects of the present invention and in fact it will be noted that in the modification shown in Figs. 8 and 9 no such mechanical interlocking is provided for. The construction shown in Figs. 8 and 9 is essentially similar to the construction shown and described in the preceding figures. In other words, the stem 10" corresponds with the stem 10 previously shown and described and similarly too it includes an end wall 12" and projection 17" in its initial stages. Likewise the head portion 20" is provided with a bore 22" for reception of the stem 10" and this bore 22" opens into a pocket 24". In this case the pocket 24" is of a different contour than the pocket 24 previously described, this being primarily because of the fact that the shape of the final valve head is somewhat different from the construction shown in the preceding figure. The function of the various elements of the construction, the method of assembly and steps of operation to provide the completed valve are substantially the same as that previously described and for that

reason it is not believed necessary to repeat them. Neither the head 20" or stem 10" are provided with grooves such as the grooves 26 and 40 previously described, the bond of the material 30" being relied upon entirely for securing the head 5 and stem against axial separation. One difference, however, may be noted that in the construction shown in Fig. 9 a layer 42 of material which may be equivalent to any of the specific compositions of matter set out for the material 10 10 15 20 may be applied over that portion of the head 20" which is to serve as the valve seating surface, the purpose of the material 42 in this case being to provide such valve seating surface that will resist the corrosive and erosive effects of the 15 hot exhaust gases of an internal combustion engine in which the valve is to be employed. The material 42 may be added by applying it to the head 20" by welding it in place in accordance with well known practices or may be applied in 20 any other suitable manner.

Formal changes may be made in the specific embodiment of the invention shown and steps of operation described without departing from the spirit or substance of the broad invention, the 25 scope of which is commensurate with the appended claims.

What is claimed is:

1. A valve blank comprising an independently formed hollow head portion and an independently formed hollow stem portion, an end wall 30 at one end of said stem portion, said end of said stem projecting into said head portion to form a joint between them, and said stem portion having openings therethrough adjacent said end wall 35 to provide communication between the interior and exterior thereof within the area of said joint.

2. A valve blank comprising an independently formed hollow head portion and an independently formed hollow stem portion, an end wall 40 at one end of said stem portion, said end of said stem projecting into said head portion to form a joint between them, said stem portion having openings therethrough adjacent said end wall to provide communication between the interior and exterior thereof within the area of said joint, and said head portion having an annular groove 45 therein within the area of said joint.

3. A valve blank comprising an independently formed hollow head portion and an independently formed hollow stem portion, an end wall at one end of said stem portion, said end of said stem projecting into said head portion to form a joint between them, said stem portion having openings therethrough adjacent said end wall to 50 provide communication between the interior and exterior thereof within the area of said joint, and said stem portion having an annular groove 55 therein within the area of said joint.

4. In the manufacture of a hollow poppet valve, 60 the steps of forming a head portion of a size in excess of the dimensions of the head in the desired completed valve, operating upon said head portion to form a pocket therein and opening leading into said pocket, separately forming an 65 independent hollow stem portion to provide an end wall therein and a hole through a side wall thereof adjacent said end wall, inserting that end of said stem portion having said end wall into said opening to a position where said hole 70 is within the longitudinal limits of said opening, welding said head portion to said stem portion about the outer margins of said opening whereby to temporarily seal and secure said head portion to said stem portion, inserting a mass of solid 75

bonding material having a melting point lower than the melting point of the material of both said portions into said stem, heating said assembly to a temperature sufficient to render said bonding material fluid but less than the melting points of the head portion and stem portion, spinning said assembly about its axis while said bonding material is fluid whereby to centrifugally discharge said material through said hole and distribute it throughout the joint between said portions, continuing said spinning until said material has solidified, and then machining the resulting assembly.

5. In the manufacture of a hollow poppet valve, the steps of providing a hollow head having an opening leading into the interior thereof, inserting a hollow stem having an end wall and openings through the side walls thereof adjacent said end wall into said opening with said end wall within said head and said openings closed by the walls of said opening, placing a mass of solid material having a lower melting point than that of said head and stem in said stem, heating the resulting assembly to a temperature sufficient 15 to melt said material but insufficient to melt said head and stem, and then spinning said assembly about its axis whereby to cause

said molten material to be discharged through said openings in said stem and to fill the space between said stem and the walls of said opening in said head, and continuing said spinning until said material has solidified.

6. In the manufacture of a hollow poppet valve, the steps of providing a hollow head having an opening leading into the interior thereof, inserting a hollow stem having an end wall and openings through the side walls thereof adjacent 10 said end wall into said opening with said end wall within said head and said openings closed by the walls of said opening, placing a mass of solid material having a lower melting point than that of said head and stem in said stem, heating 15 the resulting assembly to a temperature sufficient to melt said material but insufficient to melt said head and stem, and then spinning said assembly about its axis whereby to cause said molten material to be discharged through said openings in 20 said stem and to fill the space between said stem and the walls of said opening in said head, continuing said spinning until said material has solidified, and then removing said end wall in said stem.

25  
GEORGE CHARLTON.